

Dec. 4, 1934.

F. J. TONE

1,982,710

REINFORCEMENT OF HIGH SPEED ABRASIVE WHEELS

Filed May 25, 1929

Fig. 1.



Fig. 2.



INVENTOR  
FRANK J. TONE

BY

Thomas C. MacKay  
ATTORNEY

## UNITED STATES PATENT OFFICE

1,982,710

REINFORCEMENT OF HIGH SPEED  
ABRASIVE WHEELSFrank J. Tone, Niagara Falls, N. Y., assignor to  
The Carborundum Company, Niagara Falls,  
N. Y., a corporation of Pennsylvania

Application May 25, 1929, Serial No. 366,034

8 Claims. (Cl. 51—206)

This invention relates to the lateral reenforcement of abrasive wheels and particularly to lateral reenforcements in which the reenforcement can be worn away automatically during the 5 grinding process or may be easily removed by the occasional application of a tool while the wheel is in operation. Another type of reenforcement for abrasive wheels has been described in co-pending U. S. application Serial No. 313,087, filed 10 October 17, 1928, and also in co-pending application Serial No. 336,557, filed January 31, 1929 (these two applications 313,087 and 336,557 have been replaced by Serial No. 445,367 filed 15 April 18, 1930). The present application differs from these co-pending applications principally in the method of applying the lateral reenforcements to the wheels and in the manner of removal of the said reenforcements.

Lateral reenforcements are intended particularly for wheels which are used at speeds greater than the usual peripheral speeds of 5500 to 6500 feet per minute, as for example, 9000 feet per minute. It has been found that the diameter of a rapidly revolving abrasive wheel becomes greater than the diameter of that same wheel at rest. This actual increase in diameter is due to centrifugal force and is consequently a function of the square of the linear velocity of the wheel for a given radius. 20 If the centrifugal force set up in the revolving wheel is great enough to strain the abrasive material beyond its elastic limit, it is almost certain to cause the wheel to burst, because the elastic limit and point of failure are very close in abrasive materials, particularly in the case of vitrified articles.

As in the case of the co-pending applications referred to, an abrasive wheel to be protected is provided with lateral reenforcements, which is accomplished by applying to one or both faces of the wheel, a reenforcement which elongates much less under a stress than the abrasive wheel does under the same stress. The latter of the above mentioned co-pending applications describes a method of reenforcement of abrasive wheels by cementing metal strengthening members to each side of the wheel by means of a cement of such thickness and characteristics that together with the metal it forms a substantial reenforcing member which prevents the increase in the diameter of the wheel beyond the elastic limit of the wheel under ordinary use.

I have, so far, described the desirable features which are the object of lateral reenforcements for abrasive wheels. In considering the type of

lateral reenforcement which is to be used in the particular case, such matters as the ease of application of the reenforcement and the ease with which it can be removed should be considered. In the case of metal rings or disks it is necessary to center the reenforcements with considerable care. There are, also, certain difficulties in removing such reenforcements, for example, the actual use of the wheel must be interrupted and a period of three to ten minutes taken to remove the unnecessary outer portions of the reenforcement. The invention described below provides means to eliminate the interruption of the operation of the wheel and the loss of time in removing reenforcements.

I have invented the following methods which I believe are characterized particularly by the ease by which the reenforcements may be applied and removed respectively.

These methods are illustrated by the accompanying drawing in which:

Figure 1 represents a side view of an abrasive wheel which has been reinforced by the application of a spray of liquid metal at high pressure; and

Figure 2 is a section of Fig. 1 taken on the line 2—2.

The process referred to will be considered in detail. In applying metal reenforcements by my method I may use spraying or electrodeposition or combinations of these processes. For example, an abrasive wheel may be sprayed with copper, brass or other suitable material in a thin coating. If desired this coating may be thickened by electrodeposition of such metals as copper, nickel, chromium, etc., the strength of which can be further increased by annealing or burnishing or both.

The material is applied by means of a metal-spraying gun. Metals which can be obtained in wire form and which can be readily melted by means of an oxyacetylene flame are used. The molten metal is driven at such a pressure into the pores of the abrasive wheel that it forms a very firmly adhering coat. Such coatings strengthen the wheels and make it possible to run them at increased speed, the increase in speed greatly depending, as would be expected, on the metal used, its thickness, etc.

A sufficient coating may be applied in about five minutes on each face of the abrasive wheel. Care is exercised that the least possible heat shock is given to the abrasive material. In fact it is better to warm the wheel up slowly before spraying and cool slowly afterwards.

In Fig. 1 a metal reenforcement is shown covering part of the lateral surface of an abrasive wheel. The portion 4 of the lateral surface of the abrasive wheel is shown with the metal re-enforcement removed. The abrasive wheel is shown as mounted on a shaft 5 with the aid of a lead bushing 8.

As the wheel wears down it may be necessary to remove a portion of the lateral reenforcement. 10 This may be done by means of a lathe tool. In some cases, however, this may not be necessary, especially if the reenforcement does not extend an appreciable thickness outside of the abrasive wheel, but is largely confined to the metal which 15 has penetrated the pores of the wheel.

While I have described certain metallic materials for use in depositing metal reenforcements, other materials, such as chromium or iron, may be applied by suitable combinations of spraying 20 and electrodeposition.

Among the advantages of my method, as above described, may be noted:

1. The reenforcement may be removed by a tool while the abrasive wheel is in operation.

25 2. The reenforcement may be automatically removed in the process of operation of the wheel without the use of a dressing tool.

3. The sprayed metal reenforcement can be applied in a very short time as compared with 30 the amount of time required to apply cementing materials.

I claim:

1. As a new article of manufacture a unitary abrasive wheel having a lateral reenforcement rigidly rooted in a side of the wheel, said reenforcement consisting of metal which fills the pores of the wheel adjacent the lateral surface and extends over said surface, and which wears away in 35 the ordinary process of peripheral grinding by 40 reason of the integral connection of the metal with the side of the wheel.

2. A method of laterally reenforcing a unitary abrasive wheel which comprises depositing metal in the pores adjacent a lateral surface and on the 45 lateral surface to form a continuous layer of metal rooted in the abrasive.

3. The step in the method of providing lateral reenforcements for unitary abrasive wheels used for peripheral grinding, which step comprises spraying one or both sides of the unitary wheel with initially molten metal driven under pressure into the superficial pores, and building up the lateral reenforcement by further spraying. 80

4. The steps in the method of providing lateral reenforcement for unitary abrasive wheels used for peripheral grinding, which steps comprise warming the unitary abrasive wheel slowly, spraying one or both sides of the wheel with initially molten metal driven under pressure into the superficial pores, building up the lateral reenforcement by further spraying, and slowly cooling the 85 wheel. 90

5. The steps in the method of providing lateral reenforcements for unitary abrasive wheels used for peripheral grinding, which steps comprise spraying one or both sides of the unitary wheel with finely divided metal and thickening the deposit by electrodeposition of metal on the sprayed coating. 95

6. The method of providing lateral reenforcements for unitary abrasive wheels used for peripheral grinding, which method comprises spraying one or both sides of the unitary wheel with finely divided metal, thickening the deposit by electrodeposition of metal on the sprayed coating, and annealing the coating. 100

7. A unitary abrasive wheel having a lateral reenforcement for one or both sides of the wheel, said reenforcement comprising a layer of metal rooted in the superficial pores of the reenforced surface by spraying molten metal against the 110 abrasive surface, and an additional layer of metal electro-chemically deposited on the sprayed coating. 110

8. A unitary abrasive wheel including a porous body of bonded abrasive grain and a lateral re-enforcement in adherent contact with a side surface of the body of the wheel, said reenforcement comprising a layer of metal driven into the pores of said body so as to wet or give the effect of wetting the surface thereof. 115

FRANK J. TONE.

60

125

65

130

70

135

75

140

80

145

85

150